

3,337,652  
**MODIFICATION OF STEREOREGULAR  
POLYOLEFINS**  
Jack J. Press, 12-18 E. Laurelton Parkway,  
Teaneck, N.J. 07666  
No Drawing. Filed Oct. 26, 1964, Ser. No. 406,631  
6 Claims. (Cl. 260—895)

The invention described herein may be manufactured and used by or for the Government of the United States of America for governmental purposes without the payment of any royalties thereon or therefor.

This application is a continuation-in-part of my copending application Ser. No. 113,972, filed April 4, 1961.

The invention relates to stereoregular polyolefins. More particularly, this invention relates to polymeric compositions having improved affinity for dyes, said compositions containing a major amount of stereoregular polyolefins.

It is known that polyethylene is vastly unsuitable for the production of textile fibers due to the relatively poor properties imparted to the product. For one thing, staple polyethylene fiber will not hold a crimp and this is necessary for textile processing. For another, it is useless to make a textured or stretch yarn from continuous filament polyethylene yarn because the characteristics imparted to the yarn are not maintained during weaving, dyeing, or ordinary use. Further, the material from which a fabric is made must be thermally stable before it may be subjected to ordinary use. It must not have a relatively low melting point, and the final fabric must not have a high degree of heat sensitivity, nor relatively soft mechanical properties at elevated temperatures. However, the thermal properties of a polyethylene fabric are such that it is impossible to subject it to ordinary ironing without physically damaging the fabric and it has been found to shrink in the conventional dryer. As is apparent from the foregoing, polyethylene cannot be utilized in the manufacture of everyday fabrics for ordinary use.

In recent times, it has been found that certain linear crystalline hydrocarbon polymers containing stereoregular macromolecules and having melting points between 150° and 300° C. can be used for the production of textile fibers without the inherent difficulties encountered with the use of polyethylene polymers for this purpose. Aside from melting point differences, polypropylene with a tertiary carbon and a methyl side chain, crystallizes differently and has a much higher resilience and elasticity. These properties are essential in generally useful textile fiber. Further, polymers of olefinic hydrocarbons containing stereoregular macromolecules, such as polypropylene, polymethylpentene, and polymethylbutene, offer considerable advantages in the production of fibers, particularly because of their good mechanical properties and light weight. However, such polymers have not been satisfactory because of their poor affinity for dyes, this poor affinity being due to the particular chemical nature of such polyolefinic hydrocarbons.

Many processes have been proposed in order to improve the affinity of such polyolefinic hydrocarbons for dyes, such as the addition of soluble solid substances to the molten polyolefin before spinning. The addition of basic substances facilitates dyeing with acid dyes, whereas the addition of acid substances favors dyeing with basic dyes. However, such processes have not been completely satisfactory because soluble modifiers interfere with crystallization, impair strength and thermal stability, and are not sufficiently available in the amorphous regions where dyeing takes place.

It has also been proposed to increase the affinity of dyes for polyolefin fibers by grafting monomers onto the fibers after subjecting the fibers to a preliminary peroxida-

tion or to high energy radiation. When such processes are applied to the polyolefin after it is in filamentary form the surface properties of the grafted fibers are considerably modified and the dye receptivity is improved. However, when such processes are applied to highly crystalline filaments, any grafting onto the preformed fibers takes place only at the surface. Therefore, subsequent dyeing is limited to the surface portion of the fiber and the dye does not penetrate inside the fiber.

In my copending application titled Modification of Stereoregular Polyolefins With Hydrophilic Copolymers, Ser. No. 400,612, filed Sept. 30, 1964, I teach that the affinity of polyolefins for dyes may be enhanced through the use of selected hydrophilic, nonsoluble copolymers consisting of oxygen containing N-heterocyclic monomeric units in combination with neutral ethylenically unsaturated monomeric units. The level of addition ranges from 2 to 20% by weight based on the polyolefin.

Now, I have discovered that the affinity of polyolefins for dyes may be further improved, over and above the improvement achieved with the above polymeric materials, if the modifier incorporated in the polyolefin is one of a specified class of copolymers in combination with selected class of secondary polar additives. Surprisingly, I have found that even at low levels of addition, I obtain synergistic improvements in dyeability by replacing between 5% and 50%, preferably only up to 25%, of the above primary hydrophilic copolymeric modifiers with selected liquid, wax, or polymeric secondary polar modifiers having negligible dyeability by themselves.

These secondary polar modifiers are generally low molecular weight additives or possess melting points somewhat lower than the polyolefin itself. These secondary additives associate themselves with the primary hydrophilic polymeric modifier in such a way as to give synergistic combinations that are fusible at temperatures not exceeding the temperature of processing of the polyolefin (150° C. to 350° C.) and have improved processability and dyeability.

As an added advantage, the use of the secondary polar additives improves brightness and clarity of the final film or luster and brightness of the final fiber. The whiteness of the fiber is also improved because a smaller amount of the primary polymeric modifier, which is responsible for the off-white color, is utilized. There is also an improvement in the ease and uniformity of dispersion of the composition. There is less blockage of filters and spinnerette holes by the composition and this tends towards an improvement in processability. An economic advantage is also associated with the use of the present composition for a smaller amount of the more expensive primary polymeric modifier is utilized in the composition while still maintaining or improving the affinity of the composition for dyes.

It is therefore an object of this invention to provide polymeric compositions having improved affinity for dyes devoid of difficulties of the prior art.

Included in this invention are stereoregular polyolefin structures with increased affinity for dyes comprising a matrix of a stereoregular polyolefin taken from the group consisting of (a) polypropylene, (b) polymethylpentene, and (c) polymethylbutene, said matrix having dispersed therein between 2 and 20% of a synergistic combination consisting of:

(1) 50 to 95% of a modifying copolymer which is hydrophilic, non-soluble in the polyolefin, and fusible at a temperature between 150° C. and 350° C., said modifying copolymer being selected from the group consisting of:

(a) 30 to 70% N-vinyl pyrrolidone/30 to 70% vinyl acetate,

- (b) 60% N-vinyl pyrrolidone/40% vinyl methyl ether,  
 (c) 80% N-vinyl pyrrolidone/20% styrene,  
 (d) 70% N-vinyl pyrrolidone/30% ethyl acrylate,  
 (e) 70% N-isoprenyl pyrrolidone/30% ethylene oxide,  
 (f) 60% N-acryloyl pyrrolidone/40% ethyl acrylamide,  
 (g) 50% N-vinyl methylpyrrolidone/50% vinyl methyl ether,  
 (h) 60% N-vinyl oxazolidone/40% acrylonitrile,  
 (i) 70% N-vinyl oxazolidinone/30% hydroxypropyl methacrylamide,  
 (j) 50% N-vinyl methyloxazolidinone/50% vinyl acetate,  
 (k) 60% N-vinyl morpholinone/40% methyl acrylate, and  
 (l) 90% N-vinyl pyrrolidone/10% ethylene,  
 all said percentages being percent by weight; and  
 (2) 5 to 50% of a lower molecular weight organic substance having at least one alkyl group with 6 to 30 carbons, said substance selected from the group consisting of:  
 (a) alkyl esters of polyhydroxy compounds,  
 (b) alkyl esters of polyglycols, 60 to 4000 M,  
 (c) alkyl ethers of polyglycols, 60 to 4000 M,  
 (d) alkyl ethers of polyhydroxy compounds,  
 (e) alkoxylated alkyl amines,  
 (f) di (2-ethylhexyl) phosphoric acid,  
 (g) stearyl phosphoric acid,  
 (h) salts of dodecylbenzene sulfonic acid,  
 (i) salts of naphthalene sulfonic acid,  
 (j) N-lauryl trimethylene diamine, and  
 (k) salts of di (2-ethylhexyl) phosphoric acid,  
 said synergistic combination being fusible at a temperature of processing of the polyolefin (150° to 350° C.) and forming a complex in said polyolefin.  
 The stereoregular polyolefins which may be used within the concept of this invention include isotactic and syndiotactic polyolefins. These materials are usually made by utilizing stereo-specific catalysts which give polymers which are substantially linear and which develop a high degree of crystallinity.  
 A preferred class of my primary polymeric modifiers consists of copolymers derived from oxygen containing N-alkenyl heterocyclic monomers, particularly alkenyl substituted lactams, oxazolidone, oxazolidinone and morpholinone monomers. This class of polymers is highly desirable because it has little or no basicity and has very high levels of affinity for a wide range of dyes. My preferred primary modifiers are neutral or only very slightly basic and yet in polyolefins, surprisingly, have higher dability with anionic (acid) dyes than the much more basic polymeric modifiers. In these monomers and polymers, the alkenyl substituted nitrogen is part of an internal amide group and is essentially neutral. Additional ring and substituted oxygen containing groups are more acidic than the substituted amide nitrogen and further reduce basicity.  
 The secondary polar additives which may be used with the primary modifier to give synergistic combinations include the following:  
 (1) Alkyl esters of polyhydroxy compounds such as:  
 (a) glycerol monostearate,  
 (b) glycerol distearate,  
 (c) glycerol tristearate,  
 (d) glycerol mono/dilaurate,  
 (e) sorbitan monostearate, and  
 (f) sorbitan dilaurate.  
 (2) Alkyl esters of polyglycols (M 60 to 4000) such as:  
 (a) ethylene glycol monostearate,  
 (b) polyethylene glycol 200 monostearate,  
 (c) polyethylene glycol 200 distearate,  
 (d) polyethylene glycol 4000 distearate,  
 (e) propylene glycol monostearate,  
 (f) polypropylene glycol 600 monoocotate,  
 (g) butylene glycol monostearate,  
 (h) polybutylene glycol 800 monostearate,  
 (i) hexylene glycol monoocotate,  
 (j) hexylene glycol adipate, and  
 (k) poly(hexylene glycol adipate) 800 to 5000 M.  
 (3) Alkyl ethers of polyglycols (60 to 4000 M) such as:  
 (a) ethylene glycol monostearyl ether,  
 (b) ethylene glycol monolauryl ether,  
 (c) polyethylene glycol 200 monostearyl ether,  
 (d) polyethylene glycol 200 monolauryl ether,  
 (e) polyethylene glycol 200 distearyl ether,  
 (f) polyethylene glycol 200 monononylphenol ether,  
 (g) polyethylene glycol 4000 monostearyl ether,  
 (h) polyethylene glycol 4000 distearyl ether,  
 (i) propylene glycol monostearyl ether,  
 (j) propylene glycol monolauryl ether,  
 (k) polypropylene glycol 600 monolauryl ether,  
 (l) butylene glycol monostearyl ether,  
 (m) hexylene glycol monoocetyl ether.  
 (4) Alkyl ethers of polyhydroxy compounds such as:  
 (a) glycerol monostearyl ether,  
 (b) glycerol distearyl ether,  
 (c) glycerol dilauryl ether,  
 (d) glycerol dihexyl ether,  
 (e) sorbitan monostearyl ether, and  
 (f) sorbitan diethyl ether.  
 (5) Alkylated amines such as:  
 (a) tertiary stearyl amine with 15 moles ethylene oxide,  
 (b) tertiary stearyl di (hydroxyethyl) amine,  
 (c) tertiary stearyl di (hydroxypropyl) amine,  
 (d) tertiary stearyl di (hydroxybutyl) amine,  
 (e) tertiary lauryl di (hydroxypropyl) amine,  
 (f) tertiary lauryl amine with 15 moles of ethylene oxide,  
 (g) tertiary stearyl amine with 15 moles of propylene oxide,  
 (h) quaternary stearyl di (hydroxyethyl) methyl ammonium sulfate,  
 (i) quaternary stearyl di (hydroxyethyl) methyl ammonium chloride, and  
 (j) quaternary stearyl methyl ammonium chloride with 15 moles of ethylene oxide.  
 (6) Alkyl phosphoric acids and salts such as:  
 (a) di (2-ethylhexyl) phosphoric acid,  
 (b) sodium salt of di (2-ethylhexyl) phosphoric acid,  
 (c) potassium salt of di (2-ethylhexyl) phosphoric acid,  
 (d) isopropyl amine salt of di (2-ethylhexyl) phosphoric acid,  
 (e) triethanolamine salt of di (2-ethylhexyl) phosphoric acid,  
 (f) monostearyl phosphoric acid,  
 (g) potassium salt of monostearyl phosphoric acid,  
 (h) distearyl phosphoric acid,  
 (i) sodium salt of distearyl phosphoric acid,  
 (j) monolauryl phosphoric acid,  
 (k) lauryl ethyl phosphoric acid, and  
 (l) diethyl phosphoric acid.  
 (7) Miscellaneous compounds such as:  
 (a) N-lauryl trimethylene amine,  
 (b) N-stearyl trimethylene diamine,  
 (c) perfluoronylic acid,  
 (d) dihydrogenated tallow-methyl amine,  
 (e) stearic acid,  
 (f) alkylene (2 to 4 carbon) oxide derivatives of alkyl (6 to 30 carbons) amide,  
 (g) polyalkylene glycols having 2 to 4 carbons and 4 to 50 alkylene oxide groups.  
 (8) Alkyl and aryl sulfonic acids and salts such as:  
 (a) dodecylbenzene sulfonic acid,

- (b) sodium salt of dodecylbenzene sulfonic acid,
- (c) potassium salt of dodecylbenzene sulfonic acid,
- (d) isopropyl amine salt of dodecylbenzene sulfonic acid,
- (e) trialkanolamine salt of dodecylbenzene sulfonic acid,
- (f) lauryl sulfonic acid,

5

maintained for 2 hours. The dye samples were then rinsed, given a 10 minute 95° C. launder in the dye pot at a 20 to 1 bath to sample ratio with a 5 gram per gallon Tide detergent solution. The samples were then rinsed, dried, and judged for depth and uniformity of shades. The results of such test are set forth in the table below:

DISCS\*

|                                   | (a)         | (b)              | (c)                 | (d)       |
|-----------------------------------|-------------|------------------|---------------------|-----------|
| Percent VOOM/Va.....              | 5.....      | 4.....           | 9.....              | 14.....   |
| Percent GMS.....                  | 1.....      | 1.....           | 1.....              | 1.....    |
| Dispersibility in Polyolefin..... | Good.....   | Excellent.....   | Good/excellent..... | Good..... |
| Dyeability with:                  |             |                  |                     |           |
| (a) DLV, DO.....                  | Medium..... | Medium/dark..... | Dark.....           | Dark..... |
| (b) AMR, AR.....                  | Light.....  | Medium.....      | Medium/dark.....    | Do.....   |

\*All percentages are by weight.

- (g) sodium salt of lauryl sulfonic acid,
- (h) naphthalene sulfonic acid,
- (i) sodium salt of naphthalene sulfonic acid,
- (j) potassium salt of naphthalene sulfonic acid, and
- (k) formaldehyde condensate of naphthalene sulfonic acid.

25

The following examples set forth typical synergistic combinations of primary and secondary modifiers falling within the concept of this invention. Each is followed by results quite clearly illustrating the synergism encountered when each combination is introduced into the stereoregular polyolefin.

#### Example 1

I prepared discs of polyolefin in the following manner utilizing as modifier N-vinyl-5-methyl-2-oxazolidinone in a balanced weight fraction copolymer with vinyl acetate (VOOM/Va) (Devlex A515, Dow Chemical Co.) alone and in combination with (GMS)—glycerol monostearate.

Various percent additions, as indicated in the table which follows, were each uniformly mixed, as solutions or as finely divided solid, with separate 5 gram samples of a finely powdered (50-200 mesh) commercial, uninhibited isotactic polypropylene (molecular weight about 350,000, melting point about 170° C., melt index of 3, and isotacticity of 95%).

The mixtures were then air dried (to remove some solvent) and then heated in a drying oven at 80° C. until all of the solvent had been removed.

Each of the dried mixtures was prepared in the form of a disc in the following manner: The powder of each sample was spread uniformly in a circular shouldered Pyrex glass dish with an inside diameter of 4 inches. The dishes were then covered by an inner nesting circular shouldered Pyrex glass dish with a bottom outer separation rib projecting downwardly about 0.05 inch. The assembly weighted with a preheated 5 pound weight was then placed in an oven at 250° C. for 6 to 15 minutes. Then the weight was removed and the assembly was placed in a refrigerator at about 4° C. to cool. The assembly dishes were then separated to give a fused disc.

A portion of each of the fusion discs after water rinsing were individually placed in a separate dye pot together with 20 times its weight of distilled water and from 0.5 to 2% of the dye on the weight of the sample. The following dyes were utilized in separate baths, viz.

AMR—Colour Index, Acid Red 182,

AR—Colour Index, Acid Red 127,

DO—Colour Index, Disperse Orange 3, and

DLV—Latyl Violet 2R, Disperse Dye.

35

As indicated, an improvement in dyeability is achieved, although accompanied by a 20% reduction in the amount of copolymer utilized in the composition if a selected lower melting additive is substituted in part for the copolymer. As an added advantage, higher levels of dispersion and dyeability may be achieved with higher levels of addition. This is surprising because when the primary polymeric modifiers are utilized alone, one obtains poor dispersibility with higher levels of addition.

#### Example 2

In this example, tests similar to those of Example 1 were performed except that, in this case, the modifier containing polyolefin was extruded into fiber, drawn and then dyed using conventional equipment and processes.

The formulation was melt mixed in a continuous screw extruder, forced through a 60 mil die at 260° C. and collected at ambient temperature on a reel as a 30 denier filament.

The filament was then heat stretched 300% to give a strong, oriented 10 denier fiber. Fiber skeins were then scoured with detergent at 140° F., and dyed at the boil for one hour at 20/1 bath to fiber ratio.

The fiber, as spun, was judged subjectively for uniformity of dispersion of the modifiers in the polyolefin and the dyeings were judged for level of dyeability (depth of shade) with the following dyes:

DLV—Latyl Violet 2R, Disperse Dye,

DO—Colour Index, Disperse Orange 3,

AMR—Colour Index, Acid Red 182,

AR—Colour Index, Acid Red 127.

The synergistic combination, which was utilized as the modifier, consisted of a copolymer, 50% vinyl methyl oxazolidinone with 50% vinyl acetate (VOOM/Va), in combination with (GMS)—glycerol monostearate.

TABLE\*

|                                   | (a)              | (b)                 |
|-----------------------------------|------------------|---------------------|
| Percent VOOM/Va.....              | 4.....           | 9.....              |
| Percent GMS.....                  | 1.....           | 1.....              |
| Dispersibility in Polyolefin..... | Excellent.....   | Good/excellent..... |
| Dyeability with:                  |                  |                     |
| (a) DLV, DO.....                  | Medium/dark..... | Dark.....           |
| (b) MAR, AR.....                  | Medium.....      | Medium/dark.....    |

\*All percentages being by weight.

As indicated above, one obtains improvement in dyeability even when the combination is reduced to fiber form.

#### Example 3

In accordance with the procedure of Example 1, I prepared discs utilizing as modifier 6% by weight of a copolymer of N-vinyl pyrrolidone and vinyl acetate (70/30 weight ratio) alone, and in combination at the

60

65

70

temperature of about 95° C. and the temperature was 75

4% level with 2% by weight of the secondary additives set forth in the table below. Each of the discs was dyed following the procedure heretofore described and the finished disc was judged subjectively for uniformity of dispersion and depth of coloration. The results of these tests are tabulated below:

|     | Secondary Additive                                                        | Dispersibility in Polyolefin | Dyeability with dyes |                |
|-----|---------------------------------------------------------------------------|------------------------------|----------------------|----------------|
|     |                                                                           |                              | (a)<br>DLV, DO       | (b)<br>AMR, AR |
|     |                                                                           |                              |                      |                |
| 1.  | Blank                                                                     | Fair                         | Medium               | Medium.        |
| 2.  | Polyethylene glycol 200 nonylphenol                                       | Good/excellent               | Medium/dark          | Do.            |
| 3.  | Ethylene glycol monostearate                                              | Excellent                    | do                   | Do.            |
| 4.  | Polyethylene glycol 200 distearate                                        | do                           | do                   | Do.            |
| 5.  | Dihydrogenated tallow methyl amine                                        | Good                         | Medium               | Medium/dark.   |
| 6.  | Lauryl di (hydroxy propyl) amine                                          | Good/excellent               | Medium/dark          | Medium.        |
| 7.  | Tertiary lauryl amine with 15 moles of ethylene oxide                     | Excellent                    | do                   | Medium/dark.   |
| 8.  | Quaternary hydrogenated tallow di (hydroxymethyl) methyl ammonium sulfate | do                           | do                   | Do.            |
| 9.  | Stearyl di (hydroxy ethyl) amine                                          | Good/excellent               | do                   | Medium.        |
| 10. | Quaternary stearyl di (hydroxyethyl) methyl ammonium chloride             | do                           | Medium/dark          | Medium/dark.   |
| 11. | Tertiary stearyl amine with 15 moles ethylene oxide                       | Excellent                    | Dark                 | Do.            |
| 12. | Di (2-ethylhexyl) phosphoric acid                                         | do                           | do                   | Medium.        |
| 13. | Stearic acid                                                              | do                           | do                   | Do.            |

Note that, in all cases, the affinity of the polyolefin composition for dyes was increased by addition of a

2, the modifier containing polyolefin was extruded into fiber, drawn, and then dyed using conventional equipment and processes.

5 The synergistic combination, which was utilized as the modifier, consisted of a copolymer, 70% vinyl pyrrolidone with 30% vinyl acetate (VP/Va), in combination with

(TSA)—tertiary stearyl amine with 15 moles ethylene oxide.

TABLE\*

|                               | (a)        | (b)       | (c)         | (d)        |
|-------------------------------|------------|-----------|-------------|------------|
| Percent VP/Va                 | 2          | 4         | 9           | 8.         |
| Percent TSA                   | 1          | 1         | 1           | 2.         |
| Dispersibility in Polyolefins | Excellent  | Excellent | Good        | Excellent. |
| Dyeability with:              |            |           |             |            |
| (a) DLV, DO                   | Light      | Medium    | Dark        | Dark.      |
| (b) AMR, AR                   | Very light | do        | Medium/dark | Do.        |

\*All percentages being by weight.

selected secondary additive. In the case of the blank, the dispersibility was only fair while the depth of coloration lies in the medium range. With the addition of the selected secondary additive, the dispersibility was good to excellent and the depth of coloration was increased, in some cases, from medium to medium/dark and dark. This improvement, in all cases, is the direct result of the synergistic combination in the olefinic composition as taught by the present concept.

#### Example 4

In accordance with the procedure set forth in Example

45 As shown above, improved results can be achieved over a wide level of addition with between 10% and 33% of the selected secondary additive making up the composition.

#### Example 5

50 In accordance with Example I, I prepared discs using as modifiers the copolymers enumerated below, both alone, and in combination with selected secondary additives. The discs were dyed following the procedure heretofore described and the finished discs were judged subjectively for uniformity of dispersion and depth of color.

|     | Copolymer                                | Percent* Ratio | Percent* Addition | Secondary Additive                                      | Percent* Addition | Dispersibility in Polyolefin | Dyeability with dyes |              |
|-----|------------------------------------------|----------------|-------------------|---------------------------------------------------------|-------------------|------------------------------|----------------------|--------------|
|     |                                          |                |                   |                                                         |                   |                              | (a) DLV, DO          | (b) AMR, AR  |
| (a) | N-vinyl pyrrolidone-vinyl methyl ether.  | 60/40          | 4                 |                                                         |                   |                              | Light/medium         | Light.       |
| (b) | do.                                      | 60/40          | 4                 | Ethylene glycol monostearate.                           | 1                 | Excellent                    | Medium/dark          | Medium.      |
| (c) | N-vinyl pyrrolidone-styrene.             | 80/20          | 4                 |                                                         |                   |                              | Light/medium         | Light.       |
| (d) | do.                                      | 80/20          | 4                 | Di(2-ethylhexyl) phosphoric acid.                       | 1                 | Good                         | Medium/dark          | Medium.      |
| (e) | N-vinyl pyrrolidone-ethyl acrylate.      | 70/30          | 4                 |                                                         |                   |                              | Medium               | Light.       |
| (f) | do.                                      | 70/30          | 4                 | Tertiary stearyl amine with 15 moles of ethylene oxide. | 1                 | Excellent                    | Dark                 | Medium/dark. |
| (g) | N-isoprenyl pyrrolidone-ethylene oxide.  | 70/30          | 4                 |                                                         |                   |                              | Medium               | Light.       |
| (h) | do.                                      | 70/30          | 4                 | Ethylene glycol distearate.                             | 1                 | Excellent                    | Dark                 | Medium/dark. |
| (i) | N-acryloyl pyrrolidone ethyl acrylamide. | 60/40          | 4                 |                                                         |                   |                              | Medium               | Light.       |

|                                                                             | Copolymer | Percent*<br>Ratio | Percent*<br>Addition | Secondary Additive                                            | Percent*<br>Addition | Dispersibility<br>in Polyolefin | Dyeability with dyes |               |
|-----------------------------------------------------------------------------|-----------|-------------------|----------------------|---------------------------------------------------------------|----------------------|---------------------------------|----------------------|---------------|
|                                                                             |           |                   |                      |                                                               |                      |                                 | (a) DLV, DO          | (b) AMR, AR   |
| (j) -----do-----                                                            |           | 60/40             | 4                    | Dihydrogenated<br>tallow-methyl<br>amine.                     | 1                    | Good/excellent                  | Dark-----            | Medium.       |
| (k) -----N-vinyl oxazolidone-<br>acrylonitrile.                             |           | 60/40             | 4                    |                                                               |                      |                                 | Medium-----          | Light.        |
| (l) -----do-----                                                            |           | 60/40             | 4                    | Stearyl di-(hydroxy<br>ethyl) amine.                          | 1                    | Good/excellent                  | Dark-----            | Medium.       |
| (m) -----N-vinyl methyl<br>oxazolidone-<br>hydroxypropyl<br>methacrylamide. |           | 70/30             | 4                    |                                                               |                      |                                 | Light/medium         | Light.        |
| (n) -----do-----                                                            |           | 70/30             | 4                    | Stearic acid-----                                             | 1                    | Good/excellent                  | Dark-----            | Medium/dark.  |
| (o) -----N-vinyl morpho-<br>linone-methyl<br>methacrylate.                  |           | 60/40             | 4                    |                                                               |                      |                                 | Medium-----          | Light.        |
| (p) -----do-----                                                            |           | 60/40             | 4                    | Tertiary stearyl<br>amine with 15<br>moles ethylene<br>oxide. | 1                    | Good/excellent                  | Medium/dark          | Medium.       |
| (q) -----N-vinyl pyrrolidone-<br>ethylene.                                  |           | 90/10             | 4                    |                                                               |                      |                                 | Medium-----          | Light/medium. |
| (r) -----do-----                                                            |           | 90/10             | 4                    | Tertiary stearyl<br>amine with 15<br>moles ethylene<br>oxide. | 1                    | Good-----                       | Medium/dark          | Medium.       |

\*All percentages being by weight.

Note that the affinity of the polyolefin for dyes is increased, when one of the above selected secondary additives are utilized, in conjunction with the copolymers listed, to modify the composition of the polyolefin. This being an improvement, in all cases, over the use of the copolymer alone for the same purpose.

Many alternate methods of combining my modifiers with polyolefins are readily available. They may be combined during formation of the polymeric modifier or during actual polymerization of the polyolefin, with or without melting. They may be added to freshly polymerized polyolefin, which is still in solution in a suitable solvent, in the powdered form, or as a solution in a compatible solvent, or merely as a dispersion. They may be added to the polyolefin during precipitation, washing, neutralizing or compounding of the freshly prepared polyolefin prior to drying. This may be accomplished by adding the modifier as a powder or as a solution which is a non-solvent for the polyolefin.

The modifiers may also be melt mixed during processing or blending of the polymer prior to use in extension of fiber, film, coating or plastic. It may also be added as a liquid or powder to finely ground or micronized polyolefin polymers and then melt dispersed in situ during hot dip or spray coating or during spreading and heat coating operation. They may be incorporated in polyolefin solutions or emulsion and then applied to surfaces with or without heating.

In my copending application, I show the use of selected hydrophilic polymers to improve the dyeability of the stereoregular, high melting polyolefin. The level of addition of these primary modifiers should be between 2 and 20% of the weight of the overall composition including polyolefin. As shown and substantiated herein by the results which follow each of the examples, the utility of these primary modifiers may be vastly improved by replacing from 5 to 50%, preferably not more than 25%, of the primary modifier by a secondary modifier, heretofore listed, which has limited utility by itself.

The synergistic effects of the combinations, as taught, on the polyolefin includes vastly improved dyeability. However, the listed secondary modifiers also enhance the compatibility of the primary polymeric modifier in the polyolefin. These advantages are also accompanied by improvements in processing of the overall combination and, surprisingly, many infusible primary modifiers are rendered fusible and may be utilized within the concept of this invention to improve the dyeability of a polyolefin structure as heretofore taught.

The level of addition to the polyolefin of the synergistic combination heretofore described should be between 2 and 20% of the weight of the overall composition. If less than 2% is utilized, significant improvement will not be achieved in dyeability. If an amount greater than 20% is added to the polyolefin, many of the physical properties of the final product will be adversely affected. These include loss of strength and a lower resistance to repeated flexing.

As to the synergistic combination, it is desirable to use a minimum amount of secondary lower molecular weight additive to minimize any adverse effects on the properties of the fibers. An addition of the secondary additive above the limit stated (50%) may be in excess of that required to associate and complex with the primary modifier which makes up 50% to 95% by weight of the synergistic combination. As a result, the excess secondary additive may sweat out of the polyolefin and interfere with processing.

I prefer however to use not more than 25% by weight of the secondary polar additive, since even between 25 and 50% there might be excessive reduction in the melting point of the combination and this would result in difficulties in processing, particularly drying.

It is also preferred that the addition of the secondary additive not go below 5% by weight because below this level very little improvement is achieved in dyeability.

The primary polymeric modifier of the combination should comprise at least 25% by weight of an oxygen containing N-heterocycle monomeric unit in combination with not more than 75% of an ethylenically unsaturated monomeric unit having no basic groups. If the latter unit is present in an amount over 75%, you obtain very low levels of dyeability. It is therefore necessary to use very excessive amounts of modifier to achieve desired results.

If the ethylenically unsaturated unit is present between 50 to 75% by weight, higher levels of addition are required. The melting point of the overall composition may be reduced to such an extent that the modifier, particularly at higher levels of addition, may give some problems in processing.

However, if the latter monomeric units are present below 50% by weight of the overall primary modifier, lower levels of addition can be used to improve dyeability without processing problems resulting from an excessive reduction in melting point. This represents the optimum from a commercial point of view.

Under present concept, I prefer hydrophilic polymeric primary modifiers as part of my synergistic combination

which may be soluble in either water or an oxygenated solvent but which are not soluble in the polyolefin. I do prefer modifiers which are fusible and can be dispersed in the polyolefin.

Prior experience with comparatively less hydrophobic fiber forming polymers, such as polyacrylonitrile polymers and polyamides, have shown that the use of hydrophilic, water soluble or dispersible, modifiers is impractical. Mainly, because excessive amount of the modifier are leached out in scouring and dyeing processes. Surprisingly, I have found that my hydrophilic polymeric modifiers, when melt dispersed in the more hydrophobic polyolefin, have good dispersion stability and are not susceptible to leachage.

I have found that at comparatively low levels of addition, my synergistic combination, as taught, confers good dyeability on the polyolefin without the necessity for costly and sometimes impractical post treatments.

My hydrophilic primary polymeric modifiers must be fusible with the polyolefin. This is necessary for the formation of a continuous network of modifier throughout the polyolefin in order to permit dye penetration and efficient coordination of the dye and modifier throughout the film or fiber.

The use of a non-fusible cross-linked modifier, which results in poor dispersion, is ineffectual. The required modifier network in such a case cannot be formed and the discrete, separate particles are surrounded by unmodified areas within the polyolefin matrix. As a result, dyeing is limited to the fiber surface and the dye cannot penetrate into the interior of the fiber where it is most desired.

It is generally recognized that dyeing takes place almost entirely in the more open and readily accessible amorphous areas. When a soluble modifier is utilized, it is usually spread throughout the amorphous and crystalline areas of the polyolefin. As a result, the modifier in the crystalline areas is not available for improvement in dyeability. It also interferes with crystallization and adversely affects strength and thermal stability. However, my synergistic combination is not sufficiently compatible to be a part of the more uniform and denser crystalline areas. It appears to concentrate in the more amorphous areas where it is necessary for dyeability. It has also been found that an increase in molecular weight of my modifiers, further reduces compatibility with stereoregular polyolefins and promotes concentration of the modifier in the more amorphous regions where it may improve the dyeability of the polyolefinic matrix.

Obviously, many modifications and variations of the present invention are possible in the light of the above teaching. For instance, the synergistic combination of this invention may be used to increase opacity and the affinity of the polyolefin for finishes. They may also be used to improve the printability of the polyolefin, increase the adhesion of the polyolefin to other materials, or to reduce the overall static propensity of the final product. It is therefore to be understood that within the scope of the appended claims, the invention may be practiced otherwise than as specifically described.

I claim:

1. A polymeric composition having improved affinity for dyes consisting essentially of:

a matrix of stereoregular polyolefin taken from the group consisting of:  
65  
polypropylene,  
polymethylpentene, and  
polymethylbutene;

said matrix having dispersed therein between 2 and 20 percent by weight of a synergistic combination consisting of:

(1) 50 to 95% by weight of a modifying copolymer which is hydrophilic, non-soluble in the polyolefin, and fusible at a temperature between 150° 70  
75

C. and 350° C., said modifying copolymer being selected from the group consisting of:

- (a) 30 to 70% N-vinyl pyrrolidone/30 to 70% vinyl acetate,
- (b) 60% N-vinyl pyrrolidone/40% vinyl methyl ether,
- (c) 80% N-vinyl pyrrolidone/20% styrene,
- (d) 70% N-vinyl pyrrolidone/30% ethyl acrylate,
- (e) 70% N-isoprenyl pyrrolidone/30% ethylene oxide,
- (f) 60% N-acrylyl pyrrolidone/40% ethyl acrylamide,
- (g) 50% N-vinyl methylpyrrolidone/50% vinyl methyl ether,
- (h) 60% N-vinyl oxazolidone/40% acrylonitrile,
- (i) 70% N-vinyl oxazolidinone/30% hydroxypropyl methacrylamide,
- (j) 50% N-vinyl - 5 - methyl-2-oxazolidinone/50% vinyl acetate,
- (k) 60% N-vinyl morpholinone/40% methyl acrylate, and
- (l) 90% N-vinyl pyrrolidone/10% ethylene, said percent being by weight, and

(2) 5 to 50% by weight of a lower molecular weight polar organic substance having at least one alkyl group with 6 to 30 carbons, said substance selected from the group consisting of:

- (a) alkyl esters of polyhydroxy compounds,
- (b) alkylene amines,
- (c) fatty amides,
- (d) alkyl ethers of polyhydroxy compounds,
- (e) alkoxyLATED amines,
- (f) di (2-ethylhexyl) phosphoric acid,
- (g) stearyl ester of phosphoric acid,
- (h) salts of dodecylbenzene sulfonic acid,
- (i) salts of naphthalene sulfonic acid,
- (j) salts of di (2-ethylhexyl) phosphoric acid; said synergistic combination being fusible with said polyolefin at processing temperatures up to 350° C.

2. The composition of claim 1 wherein:

said copolymer consists of 50% by weight N-vinyl methyloxazolidinone in combination with 50% by weight of vinyl acetate, and said lower molecular weight organic substance consists of fatty esters of polyhydroxy compounds.

3. The composition of claim 1 wherein:

said copolymer consists of 30 to 70% by weight of N-vinyl pyrrolidone in combination with 30 to 70% vinyl acetate, and said lower molecular weight organic substance consists of alkoxyLATED fatty amines.

4. The composition of claim 1 wherein:

said copolymer consists of 60% by weight of N-vinyl morpholinone in combination with 40% by weight of methyl acrylate, and said lower molecular weight organic substance consists of fatty esters of polyglycols.

13

5. The composition of claim 1 wherein:  
said copolymer consists of 70% by weight of N-vinyl  
pyrrolidone in combination with 30% by weight  
of ethyl acrylate, and said lower molecular weight  
organic substance consists of fatty ethers of poly- 5  
glycols.

6. The composition of claim 1 wherein:  
said copolymer consists of 60% by weight of N-acryloyl  
pyrrolidone in combination with 40% by weight  
ethyl acrylamide, and said lower molecular weight 10  
organic substance consists of alkyl phosphoric acid.

14

## References Cited

## UNITED STATES PATENTS

3,153,680 10/1964 Guistiniani et al. \_\_\_\_ 260—897

## FOREIGN PATENTS

834,160 5/1960 Great Britain.

MURRAY TILLMAN, Primary Examiner.

D. J. BREZNER, Assistant Examiner.